

## UNITED STATES PATENT OFFICE.

EMILE BINDSCHEDLER, OF PHILADELPHIA, PENNSYLVANIA, AND GEORGE JUER, OF HOPEWELL, VIRGINIA, ASSIGNEES TO TUBIZE ARTIFICIAL SILK COMPANY OF AMERICA, A CORPORATION OF DELAWARE.

PROCESS FOR THE MANUFACTURE OF ARTIFICIAL SILK AND OTHER PRODUCTS FROM CELLULOSE ESTERS.

No Drawing.

Application filed February 24, 1922. Serial No. 538,947.

To all whom it may concern:

Be it known that we, EMILE BINDSCHEDLER, a citizen of the Republic of Switzerland, and resident of Philadelphia, in the 5 county of Philadelphia, in the State of Pennsylvania, and GEORGE JUER, recently a subject of the former Austro-Hungarian Empire, and now a resident of Hopewell, in the county of Prince George, in the State 10 of Virginia, have invented certain new and useful Improvements in Processes for the Manufacture of Artificial Silk and Other Products from Cellulose Esters, of which the following is a true and exact description.

15 Our invention relates to the manufacture of articles from cellulose esters and, particularly, to the manufacture of artificial silk therefrom. It is known that acetone and its homologues are solvents for cellulose esters but a good practical process for converting the collodion made by dissolving cellulose esters in acetone or its homologues into a clear unclouded product with economical cost of manufacture and recovery 20 25 of the solvents has not heretofore been provided. The object of our invention is to provide such a process.

Our invention consists in the process of forming clear unclouded and lustrous products, particularly artificial silk, from cellulose esters by dissolving cellulose esters in acetone or its well known homologues or mixtures thereof, imparting to the collodion thus formed the desired form, as by 30 35 forcing it through spinnerets to form artificial silk filaments and extracting the solvents from the formed filaments or other articles by immersing said product in an aqueous solution of a suitable inorganic chemical which is mixable with the acetone and in which the cellulose esters are insoluble. The extraction of the solvents can be effected by immersing the spools or bobbins on which the formed filaments are 40 45 wound in a bath of such liquid or by providing a coagulating bath of such liquid through which the formed filaments are passed.

Liquids well adapted for the removal of the acetone by our process are—certain acids, such as dilute sulphuric acid,—solution of acid salts, such as nitrecake,—or

neutral salts, for instance, and preferably a concentrated solution of calcium chloride. Such solutions mix readily with the acetone and are entirely without effect upon the cellulose esters, and from all such liquids the acetone can be readily recovered for reuse by heating the liquids and driving off the acetone. Calcium chloride is especially well adapted for use in removing the acetone because it is both very effective and very cheap.

A typical cellulose ester which we have in mind is acetylcellulose and our process is also applicable to the treatment of mixtures of such cellulose esters and nitrocellulose.

Our process can be carried out not only by the use of acetone and its homologues as solvents but also with such solvents used in admixture with other solvents such, for instance, as ethylalcohol. Such a mixture of acetone and alcohol can be obtained at low cost by the fermentation of corn in a known manner and by reason of such cheapness we prefer to use such a mixture.

In our pending application, Serial No. 425,049 filed November 17, 1920, we have described and claimed a process of securing clear unclouded filaments from a collodion formed by dissolving nitrocellulose in acetone or its homologues and extracting the solvent in a similar way to that above described and in view of said former application our present claims are limited to a process for the treatment of acetylcellulose as distinguished from nitrocellulose.

While, as we have above stated, the claims of this application are limited to the use of our described process in the treatment of acetylcellulose or its homologues, we wish to be clearly understood as intending to cover our process as applied to mixtures of such cellulose esters and nitrocellulose and a fibre or other product made from a collodion formed from such a mixture has certain valuable qualities.

Where our process is applied to mixtures of acetylcellulose esters and nitrocellulose and an artificial silk fibre is produced from the collodion the product must be denitrated by known methods as used with fibre made from nitrocellulose.

Having now described our invention,

what we claim as new and desire to secure by Letters Patent, is:

1. The method of manufacturing clear, unclouded products from acetylcellulose or its homologues which consists in dissolving the cellulose esters in a solvent made up in whole or in part of acetone or its homologues, imparting to the acetone-collodion thus formed the desired form and extracting the solvent by immersing the formed product in a concentrated solution of calcium chloride.
2. The method of manufacturing clear, unclouded silk filaments from acetylcellulose or its homologues which consists in dissolving the cellulose esters in a solvent made up in whole or in part of acetone or its homologues, imparting to the acetone-collodion thus formed the desired form and extracting the solvent by immersing the formed product in a concentrated solution of calcium chloride.
3. The method of manufacturing clear, unclouded silk filaments from acetylcellulose or its homologues which consists in dissolving the said cellulose esters in a mixture of acetone and ethylalcohol imparting to the acetone-collodion thus formed the desired form and extracting the solvent by immersing the formed product in a concentrated solution of calcium chloride.
4. The method of manufacturing clear, unclouded products from acetylcellulose or its homologues in admixture with nitrocellulose which consists in dissolving the said cellulose esters and nitrocellulose in a solvent made up in whole or in part of acetone or its homologues, imparting to the acetone-collodion thus formed the desired form and extracting the solvent by immersing the formed product in a concentrated solution of calcium chloride.
5. The method of manufacturing clear, unclouded products from acetylcellulose or its homologues in admixture with nitrocellulose which consists in dissolving the said cellulose esters and nitrocellulose in a mixture of acetone and ethylalcohol imparting to the acetone-collodion thus formed the de-

sired form and extracting the solvent by immersing the formed product in a concentrated solution of calcium chloride.

6. The method of manufacturing clear, unclouded silk filaments from acetone cellulose or its homologues in admixture with nitrocellulose which consists in dissolving the cellulose esters and nitrocellulose in a solvent made up in whole or in part of acetone or its homologues, imparting to the acetone-collodion thus formed the desired form and extracting the solvent by immersing the formed product in a concentrated solution of calcium chloride.

7. The method of manufacturing clear, unclouded silk filaments from acetylcellulose or its homologues in admixture with nitrocellulose which consists in dissolving the cellulose esters and nitrocellulose in a mixture of acetone and ethylalcohol, imparting to the acetone-collodion thus formed the desired form and extracting the solvent by immersing the formed product in a concentrated solution of calcium chloride.

8. The method of manufacturing clear, unclouded silk filaments from acetylcellulose or its homologues in admixture with nitrocellulose which consists in dissolving the cellulose esters and nitrocellulose in a solvent made up in whole or in part of acetone or its homologues, imparting to the acetone-collodion thus formed the desired form, extracting the solvent by immersing the formed product in a concentrated solution of calcium chloride and denitrating the produced filament.

9. The method of manufacturing clear, unclouded silk filaments from acetylcellulose or its homologues in admixture with nitrocellulose which consists in dissolving the said cellulose esters and nitrocellulose in a mixture of acetone and ethylalcohol, imparting to the acetone-collodion thus formed the desired form and extracting the solvent by immersing the formed product in a concentrated solution of calcium chloride and denitrating the produced filaments.

EMILE BINDSCHEDLER.  
GEORGE JUER.